

## UNITED STATES PATENT OFFICE

WALTER C. HOLMES, OF WOODBURY, NEW JERSEY, ASSIGNOR TO E. I. DU PONT DE NEMOURS & COMPANY, OF WILMINGTON, DELAWARE, A CORPORATION OF DELAWARE

## EXPLOSIVE

No Drawing.

Application filed August 31, 1929. Serial No. 389,867.

This invention relates to stabilized explosives containing nitric esters and, more particularly, to dynamites containing nitroglycerin as the principal explosive.

5 It is the practice in the manufacture of nitroglycerin explosives, or dynamites, to incorporate with the nitroglycerin a number of other ingredients. These other ingredients are in the main non-explosive by themselves and are present as absorbents for the nitroglycerin, oxygen carriers, freezing point depressants, etc. While some of the ingredients present in dynamite are chemically inert, others may have an active chemical action, particularly as promoters of hydrolysis. It has long been recognized that nitroglycerin tends to hydrolyze more or less in the presence of acids, alkalis or soluble salts. This hydrolysis tends to form small amounts of acidity, which has a very deleterious effect on the further behavior of the nitroglycerin. In order to neutralize the effects of any small amounts of acid formed, it has been customary to incorporate, with the other ingredients of dynamite, a small percentage of a substance that can combine with the acid. Such acid-neutralizing materials have been commonly termed antacids. Heretofore, materials for this purpose have included such compounds as calcium carbonate, zinc oxide and magnesium carbonate.

The present invention has as an object the production of an explosive having improved stability. A further object of my invention is an explosive comprising a new composition of materials not heretofore proposed for this purpose.

40 Other objects and advantages of the invention will be apparent at it is better understood by reference to the following specification in which its preferred embodiments are described.

45 It has been found that the incorporation of magnesium oxide as an antacid in explosive compositions of the type described herein results in unusual and more beneficial effects than compositions heretofore used. This material may be used either in the form of a precipitated magnesium oxide

or as calcined magnesite, which is the technical product, and which consists of magnesium oxide.

The use of magnesium oxide in place of materials previously used as antacids is 55 advantageous in all nitroglycerin explosives. However, there are certain types of explosives in which its incorporation is particularly desirable, because of its effect in improving the stability and keeping properties of the explosives. One type of explosive in which the use of magnesium oxide as antacid causes great improvement is that in which nitrated aliphatic compounds, containing more nitrate groups in their formulas than nitroglycerin, are substituted for a part of the nitroglycerin such nitrated products being either dissolved in, or mixed with, the nitroglycerin. Nitrated cane sugar or other nitrated sugar, is an example of 60 such a highly nitrated compound. The nitration products of the higher alcohols are other instances of such compounds, for example, nitrated sorbitol. The inclusion of such highly nitrated compounds brings 65 about a number of advantages, including an improvement in the freezing properties of the explosive. However, these nitrated compounds, possess, in general inferior stability as compared with nitroglycerin because of 70 the greater number of nitrate groups present, which molecular structure tends to make the compounds more readily hydrolyzable, and consequently less stable. The use of magnesium oxide as an ingredient with such 75 compounds will greatly increase the stability of the explosives.

80 Another kind of explosive in which the use of magnesium oxide as an antacid is of great value is that increasingly important 85 class known as ammonia gelatins, in which a part of the strength of the gelatinized explosive is obtained by the replacement of a portion of the nitroglycerin, or other 90 liquid explosive by ammonium nitrate. Very great economic advantages come from the use of such explosives. While ammonia 95 gelatins have given considerable satisfaction in use, some difficulties have been encountered from the point of view of sta- 100

bility, the instability showing itself by a tendency to leakiness in the gelatin. The use of magnesium oxide in place of antacids previously used brings a great improvement to ammonia gelatins in this respect.

One of the commonly used methods of determining the relative stability of explosives is to measure the volume of gas evolution under standard temperature conditions, the gas formed being due to decomposition reactions. Using such a method, I have determined the amount of gas evolved from definite weights of a 40% low freezing gelatin dynamite when stored at a temperature of 40° C. for a period of 13 days. With the compositions of the dynamites uniform, except that different antacids were used, in amounts of 2% each, the following volumes of gas were obtained per 100 grams of explosive:

|                     |                       |
|---------------------|-----------------------|
| Zinc oxide          | 5.0 cc.               |
| Calcium carbonate   | 6.7 cc.               |
| Magnesium carbonate | 13.0 cc.              |
| Magnesium oxide     | a fraction of 1.0 cc. |

As the gas developed may be considered as resulting from decomposition reactions, the advantages of using magnesium oxide as the antacid are plainly shown.

By way of illustrating my invention the following examples are given, in which different embodiments are described.

A gelatin dynamite containing a nitrated sugar oil may, for example, have the following composition:

|                     | Per cent |
|---------------------|----------|
| Nitroglycerin       | 28       |
| Nitrated cane sugar | 6        |
| 40 Nitrocellulose   | 1        |
| Sodium nitrate      | 50       |
| Wood pulp           | 7        |
| Starch              | 4        |
| Sulphur             | 2        |
| 45 Magnesium oxide  | 2        |

An ammonia gelatin likewise may have the following composition:

|                   | Per cent |
|-------------------|----------|
| Nitroglycerin     | 24.0     |
| 50 Nitrocellulose | 0.6      |
| Ammonium nitrate  | 10.0     |
| Sodium nitrate    | 51.0     |
| Wood pulp         | 8.0      |
| Starch            | 2.4      |
| 55 Sulphur        | 2.0      |
| Magnesium oxide   | 2.0      |

It is to be understood that the above examples are merely illustrative of explosive mixtures containing magnesium oxide as an acid-neutralizing material, and that the above compositions may vary widely both in the kinds and amounts of ingredients used.

In the examples given, I have cited nitro-glycerin as the liquid explosive ingredient.

I may, however, if desirable, replace the nitroglycerin wholly or in part by a nitro-glycol, for example, ethylene glycol dinitrate, or I may substitute for a portion of said liquid ingredient any of the recognized freezing point depressants, such, for example, as nitrated polymerized glycerin, nitrochlorhydrins, or an aromatic nitro-compound.

In like manner, the nitrated cane sugar cited is only an example of a number of nitrated aliphatic compounds that might be used, having in its structural formula more nitrate groups than nitroglycerin. Similarly, I may replace the sodium nitrate wholly or in part by other oxygen-carrying compounds, such for example, as potassium nitrate, barium nitrate, etc.

While varying amounts of magnesium oxide may be used with beneficial effects on the properties of the explosive, I prefer to use amounts not greater than 5% of the explosive by weight, since greater percentages of this ingredient have an undesirable effect in decreasing the strength of the explosive. I prefer also to use an amount of magnesium oxide not less than 0.1%, since smaller amounts do not give as great an improvement to the explosive as desired. I have found 2% of magnesium oxide to be a satisfactory amount for use.

While I have described my invention above in detail, I wish it to be understood that many changes may be made therein, without departing from the spirit of the invention and that I do not intend to be limited except as indicated in the appended claims.

I claim:

1. An explosive composition comprising a liquid explosive, nitrocellulose and magnesium oxide.
2. An explosive composition comprising nitroglycerin, nitrocellulose, and magnesium oxide.
3. An explosive composition comprising a liquid explosive containing a nitrated aliphatic compound having more nitrate groups than nitroglycerin, and magnesium oxide.
4. An explosive composition comprising a liquid explosive containing a nitrated sugar, and magnesium oxide.
5. An explosive composition comprising nitroglycerin, a nitrated sugar, and magnesium oxide.
6. An explosive composition comprising nitroglycerin, a nitrated sugar, nitrocellulose, and magnesium oxide.
7. An explosive composition comprising nitroglycerin, a nitrated sugar, nitrocellulose, one or more oxygen-carrying compounds, absorbent materials for the liquid explosive, and magnesium oxide.
8. An explosive composition comprising

nitroglycerin, a nitrated sugar, nitrocellulose, one or more oxygen-carrying compounds, absorbent materials for the liquid explosive, and an amount of magnesium oxide between 0.1 and 5.0%.

9. An explosive composition comprising a liquid explosive, nitrocellulose, ammonium nitrate, and magnesium oxide.

10. An explosive composition comprising nitroglycerin, nitrocellulose, ammonium nitrate, and magnesium oxide.

11. An explosive composition comprising nitroglycerin, nitrocellulose, ammonium nitrate, an additional oxygen-carrying compound, absorbent material for the liquid explosive, and magnesium oxide.

12. An explosive composition comprising nitroglycerin, nitrocellulose, ammonium nitrate, an additional oxygen-carrying compound, absorbent material for the liquid explosive, and an amount of magnesium oxide between 0.1 and 5.0%.

In testimony whereof, I affix my signature.

WALTER C. HOLMES.

30

35

40

45

50

55

60

65